

J. OSTRANDER,  
PACKING AND PROCESS OF PRODUCING SAME.  
APPLICATION FILED JAN. 26, 1908.

902,318.

Patented Oct. 27, 1908.

*Fig. 1.*



*Fig. 4.*



*Fig. 3.*



*Fig. 2.*



Witnesses  
John A. Fable  
Thomas H. McMeair.

Inventor  
James Ostrander,

By *Bradford & Hood.* Attorney

# UNITED STATES PATENT OFFICE.

JAMES OSTRANDER, OF INDIANAPOLIS, INDIANA.

## PACKING AND PROCESS OF PRODUCING SAME.

No. 902,318.

Specification of Letters Patent.

Patented Oct. 27, 1908.

Application filed January 25, 1908. Serial No. 412,546.

*To all whom it may concern:*

Be it known that I, JAMES OSTRANDER, a citizen of the United States, residing at Indianapolis, in the county of Marion and State 5 of Indiana, have invented certain new and useful Improvements in Packing and Process of Producing the Same, of which the following is a specification.

It has heretofore been customary to produce a packing, for piston rods and other similar parts, by taking a plurality of sheets or strips of fabric, such as canvas, asbestos, etc., coating the same with rubber or other suitable composition, and sticking together 15 the several sheets or strips into a pile or sheet which is then vulcanized, cured or otherwise treated to bring it to the proper condition. This sheet is then cut into strips or strings having a cross section which is substantially 20 square and in use the box or gland is filled with rings formed from such strips and then subjected to a compressive force in that direction of the cross section at right angles to the planes of the fabric laminæ.

25 A number of different formations have been proposed for the purpose of increasing the amount of transverse expansion which may be accomplished by the compressive force referred to, such for instance, as that 30 shown in my Patent No. 808,775. In the actual manufacture of the packing such as that shown in my above mentioned patent, if the laminæ of fabric are regularly corrugated or otherwise transversely displaced before they 35 are brought together, some difficulty is experienced in the commercial production of such packing and the object of my present invention is to provide an improved process of producing packing having the fundamental 40 characteristic of the aforesaid packing.

The accompanying drawings illustrate my invention.

Figure 1 is a perspective view of a strip of laminated packing in process of production 45 of my present product; Fig. 2 a similar view of my improved packing produced in accordance with my improved method; Fig. 3 a similar view of a packing having the characteristics of that shown in Fig. 2 but having in 50 addition a top and bottom plate or lamina of fabric which is more uniformly corrugated and applied to the main body of the packing strip after the forming compression; Fig. 4 a perspective view illustrating the manner of 55 practicing my improved process showing a suitable means for subjecting the packing to a

transverse compression in the line of one dimension of its cross section during "curing."

In order to practice my improvement in the art of producing packing I first produce 60 a strip of material, such as is shown in Fig. 1, said strip comprising a plurality of fabric laminæ 10 and interposed yieldable cement 11 capable ultimately of withstanding the 65 temperatures to which the packing is to be subjected in actual use, such for instance as rubber. This strip may be conveniently cut from a partially cured sheet built up as described and I prefer, in order to finally produce a packing strip of the usual dimensions 70 having a cross section substantially square, to make that cross sectional dimension of the strip which is parallel with the fabric laminæ somewhat greater than the cross sectional dimension at right angles to the fabric laminæ. 75 This strip is formed at a time prior to the final curing or other "setting" treatment and is then subjected to a transverse compression substantially parallel with the fabric laminæ, thus causing a thickening or 80 wrinkling of the fabric laminæ along lines substantially parallel with the length of the strip, the amplitude of the wrinkles in the fabric as a whole or in the threads of the fabric transversely of the initial planes of the 85 fabric being comparatively small. While this wrinkled condition is extant the strip is subjected to a curing operation of such character as to "set" it in its wrinkled condition, such for instance as by vulcanizing in the 90 usual manner.

I prefer to maintain the transverse compression during the curing process and for this reason the strip may be clamped between a pair of clamps 15, 15 and held therein during the vulcanizing or other curing process. After the curing has been completed it will be readily apparent that a compressive force substantially at right angles to the original compressing force will tend to 100 return the fabric laminæ to their initial condition and consequently the packing strip is capable of very considerable transverse wearing expansion, thus materially increasing its 105 life.

If desired, after the strip has been subjected to its wrinkling compression, I may apply to the top and bottom surfaces, finishing laminæ comprising fabric strips 16, 16 which have been more uniformly wrinkled and held in that condition. The application of these 110 finishing surfaces or strips may take place

either before the curing of the main body of the strip or these strips may be separately cured and applied, by cementing or otherwise, to the set strip in which the wrinkled condition has been produced.

I claim as my invention:—

1. That improvement in the art of producing a packing which comprises the subjection of a laminated strip to a compressive force substantially parallel with the laminae and transversely thereof to produce wrinkles substantially normal to the compressive force, and subjecting the packing in its wrinkled condition to a process which will cause the same to become set in wrinkled condition. 10
  2. That improvement of producing a laminated fabric-rubber packing which consists in subjecting a strip of sheet comprising a plurality of fabric-lamina and interposed rubber to a distorting pressure applied in a direction substantially parallel with the planes of the fabric to wrinkle the same transversely, and treating the packing in its wrinkled condition to a curing process to set the same. 15
  3. That improvement in the art of producing a laminated packing which comprises the subjection of the packing to a compression in one dimension of its cross section under such conditions as to wrinkle the lamina transversely and set the same in that condition. 20
  4. That improvement in the art of producing laminated fabric packing which comprises the subjection of such packing to a compressive force which decreases the lineal dimension of the fabric-lamina in one dimension transversely to the thickness of said laminae, and setting the packing in that condition. 25
  5. That improvement in the art of producing a packing which comprises the subjection of a laminated strip to a compressive force substantially parallel with the laminae and transversely thereof to produce wrinkles substantially normal to the compressive force, and subjecting the packing in its wrinkled condition to a process which will cause the same to become set in wrinkled condition and attaching thereto a previously corrugated finishing lamina. 30
  6. That improvement of producing a laminated fabric-rubber packing which consists in subjecting a strip or sheet comprising a plurality of fabric-lamina and interposed rubber to a distorting pressure applied in a direction substantially parallel with the planes of the fabric to wrinkle the same transversely, and treating the packing in its wrinkled condition to a curing process to set the same and attaching thereto a previously corrugated finishing lamina. 35
  7. That improvement in the art of producing a laminated packing which comprises the subjection of the packing to a compression in one dimension of its cross section under such conditions as to wrinkle the lamina transversely and set the same in that condition and attaching thereto a previously corrugated finishing lamina. 40
  8. That improvement in the art of producing laminated fabric packing which comprises the subjection of such packing to a compressive force which decreases the lineal dimension of the fabric-lamina in one dimension transversely to the thickness of said laminae, setting the packing in that condition, and attaching thereto a previously corrugated finishing lamina. 45
  9. As an article of manufacture, a packing strip comprising a stack of cemented fabric laminae which have been set by transverse compression substantially in the planes of laminae in an abnormal and reduced lineal dimension at right angles to their thicknesses. 50
  10. As an article of manufacture, a packing comprising a stack of fabric laminae cemented together with rubber, said stack having a lineal dimension substantially at right angles to the thicknesses of the laminae which has been reduced by transverse compression substantially in the planes of the laminae. 55
  11. As an article of manufacture, a packing strip comprising a stack of fabric laminae cemented together with a flexible cement, wherein the fabric laminae have been wrinkle transversely by a compressive force exerted in the planes of the laminae, and the packing set in its wrinkled condition. 60
- In witness whereof, I, have hereunto set my hand and seal at Indianapolis, Indiana, this 22 day of January, A. D. one thousand nine hundred and eight.

JAMES OSTRANDER. [L. s.]

Witnesses:

ARTHUR M. HOOD,  
THOMAS W. MCMEANS.